

## UNITED STATES PATENT OFFICE.

SAMUEL H. FLEMING, OF CLEVELAND, OHIO, ASSIGNOR TO NATIONAL CARBON COMPANY, OF CLEVELAND, OHIO, A CORPORATION OF NEW JERSEY.

## ARTICLE WITH PROTECTIVE COATING.

1,098,794.

Specification of Letters Patent.

Patented June 2, 1914.

No Drawing.

Application filed October 29, 1912. Serial No. 728,362.

To all whom it may concern:

Be it known that I, SAMUEL H. FLEMING, a citizen of the United States, and a resident of Cleveland, in the county of Cuyahoga, in the State of Ohio, have invented new and useful Improvements in Articles with Protective Coatings, of which the following is a clear and exact description.

My invention relates to protective coverings for electrodes, resistors, furnace bricks and similar articles.

The object of the invention is to produce a hard adhesive, non-porous coating that will stand the high temperatures attained in an electric or other furnace without burning, or undergoing other deleterious chemical changes. The manner in which this is accomplished will be given in the accompanying description.

20 Titanium nitrid is a stable compound even at very high temperatures. It is non-porous, difficult to break, and is very hard, so that it forms an efficient covering for articles of carbon or other refractory material, as it prevents the air or other furnace gases from reaching the carbon or other material to combine therewith.

To form the covering for an article a mix is made of some titanium compound, 30 such as rutile for example, and a suitable binder and this is applied to the surface of the article by any means. The mix may be forced around the article at the same time that the latter is forced, in a manner 35 similar to known process for putting thin shells around arc light electrodes, or it may be pressed on. After the article is coated with a titanium compound such as rutile, it is baked at a high temperature in the 40 presence of nitrogen. Titanium has a high affinity for nitrogen and the two readily combine to form the nitrid. By this means the coating of titanium oxide or other compound is converted into titanium nitrid.

45 In some cases it may be desirable to have the article provided with an exterior nitrid coat and an interior carbid coat, as the latter would serve as means to more firmly unite the former to the carbon. Titanium 50 carbid wets the carbon and enters the pores of its exterior surface, so that the union with the carbon is practically perfect.

Titanium carbid itself is a poor coating for articles subject to a high temperature in the presence of air, as it readily burns. 55 However, if the coat of titanium carbid is surrounded by a layer of titanium nitrid it will be protected from the air and will not burn. One of the ways in which these two coats may be applied to the article is to apply a mix containing titanium and carbon to the article as previously described and then heat the article with the exclusion of air or nitrogen and thus form titanium carbid from the union of the titanium with the carbon. After the coating of carbid is formed the article is heated in the presence of air or other nitrogen supply and part or all of the titanium carbid is converted into the nitrid. The process can be 60 stopped before the entire coat of carbid is transformed into the nitrid, if an inner 65 coat of titanium carbid is desired.

While I prefer to apply the nitrid coating in the way previously described, I may 70 use another method for forming the coating. The article itself may consist of carbon mixed with rutile or other titanium compound in the desired proportions. When this is heated the outer surface of 75 the electrodes will be converted to titanium carbid. The carbid coating may be later entirely or partially converted into the nitrid by heating in the presence of nitrogen as previously described, or the article 80 may be first heated in an atmosphere of nitrogen so that a coating of the nitrid is 85 directly formed.

Having described my invention what I 90 claim is:

1. A refractory article having a coating of titanium nitrid.
2. A refractory article having one coating of titanium carbid and a second superimposed coating of titanium nitrid.
3. A carbonaceous article, the outer portions of which contain titanium nitrid.
4. The process of forming a coating on an article which consists in applying a layer of rutile and then heating the article 100 in the presence of nitrogen.
5. The process of forming a coating on an article which consists in applying a layer of rutile and carbon, heating with

the exclusion of air to change the layer to titanium carbide, and then heating in an atmosphere of nitrogen to form titanium nitrid.

5 6. A furnace electrode consisting of carbon and having a coating of titanium nitrid to protect it from oxidation.

In testimony whereof I have hereunto signed my name.

SAMUEL H. FLEMING.

Witnesses:

I. J. ADAMS,  
H. G. GROVER.

Copies of this patent may be obtained for five cents each, by addressing the "Commissioner of Patents, Washington, D. C."